

## UNITED STATES PATENT OFFICE.

MATHIAS PETERS, OF DUISBURG, GERMANY.

## STEEL ALLOY FOR THE ROLLERS OF PILGER ROLLING MILLS.

No Drawing.

Application filed March 19, 1925. Serial No. 16,822.

*To all whom it may concern:*

Be it known that I, MATHIAS PETERS, a German citizen, and resident of 18 Menzelstrasse, Duisburg, Germany, have invented certain new and useful Steel Alloy for the Rollers of Pilger Rolling Mills, of which the following is a specification.

This invention relates to a steel alloy for the construction of the rollers of Pilger rolling mills. These rollers are subjected to considerable strain. They are also exposed to heavy and very frequent shocks. Whilst in operation it is necessary to spray them with cold water for the purpose of cooling them as otherwise they would become too hot and wear too rapidly.

In view of these conditions it is necessary to construct these rollers of a material which is extremely compact, which combines great hardness with the highest degree of toughness, which is as insensitive as possible to rapidly changing temperatures, which is therefore not liable to be cracked superficially, which in spite of these properties is not too difficult to work, and which finally is not substantially more expensive than steel as used hitherto for such and similar purposes.

The material which meets these requirements entirely and which was hitherto unobtainable consists of a steel alloy of which the essential additions consist in 1.5 to 2.2%

chromium, 1.0 to 1.65% tungsten and 1.0 to 1.65% nickel. The alloy may also contain 0.6 to 0.8% carbon, 0.4 to 0.7% manganese, 0.015 to 0.2% silicon, and phosphorus and sulphur below 0.03%.

Having thus described my invention what I claim as new and desire to secure by Letters Patent is:—

1. A steel alloy for rollers for Pilger rolling mills consisting of steel containing about 2% of chromium, about 1.5% tungsten and about 1.5% nickel.

2. A steel alloy for the rollers of Pilger rolling mills, said alloy consisting of steel containing about 2% of chromium, about 1.5% tungsten, about 1.5% nickel, about 0.7% carbon, about 0.55% manganese, about 0.1% silicon, and below 0.03% phosphorus and sulphur.

3. As an article of manufacture a roller for Pilger rolling mills consisting of a steel alloy containing 1.5 to 2.2% chromium, 1.0 to 1.65% tungsten and 1.0 to 1.65% nickel.

4. As an article of manufacture a roller for Pilger rolling mills consisting of a steel alloy containing 1.5 to 2.2% chromium, 1.0 to 1.65% tungsten, 1.0 to 1.65% nickel, 0.6 to 0.8% carbon, 0.4 to 0.7% manganese, 0.015 to 0.2% silicon, phosphorus and sulphur below 0.03%.

MATHIAS PETERS.